# EUROPEAN PATENT SPECIFICATION

(11) **EP 2 102 378 B1**
(45) Date of publication and mention of the grant of the patent: **19.06.2013**
(21) Application number: 07851993.1
(22) Date of filing: 12.12.2007
(51) Int. Cl.: C22B 21/06, C22B 9/04

(54) **METHOD AND DEVICE FOR REMOVAL OF ELEMENTS RESOLVED IN A METAL MELT**
VERFAHREN UND VORRICHTUNG ZUR ENTFERNUNG VON IN EINER METALLSCHMELZE GELÖSTEN ELEMENTEN
PROCÉDÉ ET DISPOSITIF POUR LE RETRAIT D'ÉLÉMENTS DISSOUS DANS UN BAIN FONDU MÉTALLIQUE

(30) Priority: 13.12.2006 NO 20065893
(43) Date of publication of application: 23.09.2009
(73) Proprietor: Alu Innovation AS, 7401 Trondheim (NO)
(72) Inventor: VENAAS, Karl, 1344 Haslum (NO)
(74) Representative: Hindenes, Jan-Ove
(86) International application number: PCT/NO2007/000437
(87) International publication number: WO 2008/079015

(56) References cited:
- EP-A1- 1 225 236
- WO-A1-2004/076699
- GB-A- 699 934
- GB-A- 1 010 436
- JP-A- 05 302 130
- JP-A- 11 256 251
- US-A- 2 021 365
- US-A- 4 842 643
- US-A- 5 385 601
- KHABROV M F: "An Improvement in Vacuum Refining of Aluminum Alloys", LIGHT METAL AGE, FELLOM, SAN FRANCISCO, CA, US, vol. 40, no. 10, 1 October 1982 (1982-10-01), pages 33-34, XP009125438, ISSN: 0024-3345

## Description

The present invention relates to a method as stated in the introductory part of claim 1, for removal of elements from a metal melt in a container, which melt contains a base metal and elements of undesirable constituents, in which the metal melt is heated to a level maintaining the content melted, with an electrode immersed into the container. Moreover, the invention comprises a device for removal of such elements, as stated in the introductory part of claim 1.

### Background

On treating metals, the need for cleansing of a metal for another metal arises. This relates particularly to remelting of metals with impurities of one or more other metals.

An example is at remelting of aluminium containing magnesium, Mg. To provide sufficient purity, the magnesium remnants in most cases should be removedd. Currently, this is done by
1 Adding Cl2(g), which is reacting with Mg according to the equation: Mg + Cl2 = MgCl2
2 By adding active salts reducing the Mg content.

Common to both methods is the development of MgCl2, which is a salt depositing on the melt surface together with Al2O3 slag, which is removed periodically. Such slag is transferred to melting works recovering aluminium, while the rest containing oxides, chlorides etc. normally is stored on land or is dumped at sea. This is undesirable for environmental reasons.

EP 1 225 236 discloses a continuous vacuum refining method of molten metal wherein impurities in the molten metal are eliminated by evaporation by stirring the molten metal in a molten metal stirring chamber. The elements to be removed, such as magnesium, are vaporized and subsequently condensed in a separate condenser vessel.

US 4 842 643 relates to an apparatus for purifying a melt which, besides one or more impurities to be volatilized, contains essentially a light metal such as aluminium. The apparatus comprises a vacuum processing vessel and means for vaporizing and subsequently condensing the various elements in separate condenser vessel.

WO 2004/076699 reveals a vacuum container for heating metals in which electrodes are used. The device comprises a container subjected to a vacuum. A rotating electrode is arranged in the container, producing a electric arc for supply of heat to the melt.

US 5 385 601 relates to a furnace for melting aluminium dross heated with a plasma-arch to promote vaporization of volatile components. The volatile gases having left the furnace are passed through one or more condensers.

### Object

The main object of the invention is to provide a method and a device for removal of undesirable metals from metal melts, reducing said problems. It is particularly an object to provide a method and a device for remelting aluminium containing magnesium, in which Mg is removed during the melting treatment. It is an object to provide a device being advantageously built, operated and maintained.

The invention should be integrated in a device according to Norwegian patent specification 318848, with the general scheme of operation: In a hollow rotating body being immersed in a melt, an electrode conducting gas is arranged. Between the electrode and the melt a flame arch is burning, from which the heat energy is transferred directly to the melt.

### The Invention

In the following, the method according top the invention is defined by claim 1 and the device is correspondingly defined by claim 2.

The invention may for example be used for removing of magnesium from aluminium melts.

The magnesium vapour is mixed with further gas which is added in the rotor. The gas mixture is led through a vacuum exit to a condenser for depositing of liquid magnesium. The exhaust gas from the condenser is fed through a vacuum pump into the atmosphere. The emission is without CO2 gas. If the aluminium melt contains other alkalis they will evaporate correspondingly.

### Example

The invention is described in more detail in the following and with reference to the figures, wherein
Figure 1 shows a connection between vapour pressure and temperature for some metals which could be in the melt, while
Figure 2 show a schematic side view of a plant comprising a device according to the invention, provided for removal of undesirable metals from an aluminium melt.

The example is based on a device vaporizing magnesium directly from an aluminium melt without oxidizing Al and Mg. The device is provided for bringing heat energy to the melt. In Figure 1 a diagram is showing the connection between temperature and vapour pressure for aluminium, magnesium and zinc in the range 700 - 1200 °C. The diagram shows that the vapour of aluminium in this range is negligent to the vapour pressure for the other metals.

Figure 2 shows schematically a plant with a device according to the invention. It comprises a cylindrical or rectangular upright container 1 with an outlet in the container 1 in the form of an outlet conduit 2. The melt treated flows through a tube 3 at the lower end of the outlet conduit 2. The melt to be treated is transferred via a chute to a reservoir 24 and is sucked into the lower end container 1 through a tube 4 and is lifted by a sub pressure into the container provided by a vacuum pump 29.

The vacuum pump 29 is connected to a series of three condensers 27 being connected to the container 1 by a tube 5. In the container 1, a rotor 6 is provided, powered by a motor 7 over a drive belt 8 or similar, to a pulley 9 attached to a tubular shaft connected to the rotor 6. The motor is attached to a bracket 11. The bracket 11 can be attached to the container 1 or to a separate rack. The sealing between the rotor shaft 10 and the container 1 is

provided by a sealant 12. The bracket 11 has a bearing 16 journaling the rotor shaft 10. Centrally in the shaft an electrode 13 is arranged, the upper end of which is connected to a cable with a cable shoe 14. The electrical current, which can be DC or AC, is transferred to the device through the cable shoe 14 and through an electrode connection 28 on the container 1.

The metal melt of the example is heated to a temperature between 800. and 1200 °C, preferably ca. 1000 °C by the electrode 13 and 26.

The electrode 13 has a central bore for supplying gas from a connection 15 at the outer end of the electrode 13. The gas supplied through the electrode 13 is preferably argon or nitrogen or a mixture thereof. Other gases may also be utilized. The gas over an upper melt level 21 will comprise of a mixture of gas supplied to the rotor and gas emitted from the melt. The gases emitted from the melt are hydrogen and the vapour of magnesium, zinc, sodium etc. The gases overthe melt level 21 are extracted through the tube 5 to the condensers 27, in which magnesium, zinc and sodium etc. are condensed to melts. The residual gas is fed through the vacuum pump 29 to the environment, possibly through a purification device.

Between the rotor shaft 10 and the electrode 13 a ring 16 is arranged for acting as a sealant and an electrical insulation. The ring 16 has a passage for gas and particles through a tube 17 connected to a powder supply 18. The reservoir 24 has a dividing wall 20 and a gatevalve 19 (the operation of which is not illustrated), to allow continuous handling of the melt, but the reservoir may also be a melting pot filled with melt. At the lower end of the rotor 6, multiple holes 25 are arranged between the circumference and the melt level 23. The level 23 of the melt in the rotor is governed by the gas pressure of the rotor 6.

The plant is started with the gate valve 19 closed and the reservoir 24 is filled to a certain level. When the vacuum is provided by the vacuum pump 29 through the condensers 27 and the tube 5, gas is provided simultaneously through the electrode 13 and/or the ring 16 to the rotor 6. The melt is brought to the level 21. The rotor 5 is operated and the voltage from a rectifier or transformer is applied. The current is led through the cable shoe 14 to the electrode and through the contact 28, alternatively through the rotor shaft 10 via a collector ring (not shown). A flame arch 22 is created between the electrode 13 and the top level of the melt 23. The rotation of the rotor 6 will pump the heated melt in the rotor through the holes 25 and mix it into the melt of the container. Simultaneously gas bubbles are created at the outlet of the holes 25. The gas bubbles, containing gases emitted from the melt, hydrogen and vapours of magnesium, zinc, sodium, etc. The gas bubbles are rising in the melt, through the upper level 21 and are released through the tube 5 and to the condensers 27, wherein magnesium, zinc and sodium etc. are condensed to melts which can be drained through the valve connection 30. The holes 25 of the rotor 6 can be circular or polygonal, and be arranged at the lover end of the rotor, being notches therein. When the melt has reached a desirable temperature, the valve 19 is opened and the metal may exit from the container 1 for further processing.

The invention is not restricted to the example of Figure 2. Thus, the plant can comprise two, three or more containers in a series. Each container may have multiple rotors with a flame arch.

## Claims

1. Method for removal of elements from a metal melt in a container, which melt contains a base metal and elements of undesirable constituents, in which the metal melt is heated to a level maintaining the content melted, with an electrode immersed into the container, **characterized in that** the metal melt is heated to a level causing vaporization of an element to be removed, but under the level providing gas pressure for the base metal, and that the container with the metal melt is brought under a reduced pressure in at least one compartment in which the temperature is maintained under the vaporization level of the element to be removed, and **in that** the gas is transported through a cascade arrangement with declining temperature in succeeding steps of the cascade.

2. Device for the removal of elements from metal melts, with a container (1) for the metal melt, which comprises a flame arch (22) for providing heat, and with an exit tube (5) over the level of the metal melt, for vapour from the interior of the container (1), **characterized in that** the exit tube (5) exits into a compartment (27) which is kept at a temperature under the vaporization temperature, for condensing the vaporized metal, and **in that** multiple compartments (27) with declining temperature are arranged in a series, for condensing different metal vapours, the metal with the highest vaporization point is condensed in the first compartment (27) and the metal with the lowest vaporization point is condensed in the last chamber.

## Patentansprüche

1. Verfahren zum Entfernen von Elementen aus einer Metallschmelze in einem Behälter, wobei die Schmelze ein Grundmetall und Elemente unerwünschter Bestandteile umfasst, wobei die Metallschmelze im Behälter auf ein Niveau erhitzt wird bei dem der Inhalt geschmolzen bleibt, mit einer in den Behälter eingetauchten Elektrode,
**dadurch gekennzeichnet,**
**dass** die Metallschmelze auf ein Niveau erhitzt wird, bei dem das zu entfernende Element verdampft, aber unter dem Niveau für den Gasdruck des Grundmetalls,
**dass** der Behälter mit der Metallschmelze unter einen verringerten Druck in wenigstens einem Raum, in dem die Temperatur unterhalb des Verdampfungsniveaus des zu entfernenden Elements gehalten wird, gesetzt wird, und
**dass** das Gas durch eine Kaskadenanordnung mit abnehmender Temperatur in aufeinanderfolgenden Stufen der Kaskade transportiert wird.

2. Vorrichtung zum Entfernen von Elementen aus einer Metallschmelze, mit einem Behälter (1) für die Metallschmelze, der einen Flammenbogen zur Bereitstellung von Wärme umfasst, und mit einem Ableitungsrohr (5) oberhalb des Pegels der Metallschmelze für den Dampf aus dem Inneren des Behälters (1),
**dadurch gekennzeichnet, dass**
das Ableitungsrohr (5) in einen Raum (27) führt, der auf einer Temperatur unterhalb der Verdampfungstemperatur zum Kondensieren des verdampften Metalls gehalten wird, und dass mehrere Räume (27) mit abnehmender Temperatur in einer Reihe zum Kondensieren unterschiedlicher Metalldämpfe angeordnet sind, wobei das Metall mit dem höchsten Verdampfungspunkt in dem ersten Raum (27) und das Metall mit dem niedrigsten Verdampfungspunkt in dem letzten Raum kondensiert wird.

## Revendications

1. Procédé pour le retrait d'éléments d'un bain de métal liquide dans un récipient, lequel bain contient un métal de base et des éléments de constituants indésirables, dans lequel le bain de métal liquide est chauffé à un niveau maintenant le contenu liquide, avec une électrode immergée dans le récipient, **caractérisé en ce que** le bain de métal liquide est chauffé à un niveau provoquant la vaporisation d'un élément à retirer, mais sous le niveau fournissant la pression gazeuse pour le métal de base, et **en ce que** le récipient avec le bain de métal liquide est amené sous une pression réduite dans au moins un compartiment dans lequel la température est maintenue sous le niveau de vaporisation de l'élément à retirer, et **en ce que** le gaz est transporté par un agencement en cascade avec une diminution de la température dans les échelons successifs de la cascade.

2. Dispositif pour le retrait d'éléments de bains de métal liquide, avec un récipient (1) pour le bain de métal, qui comprend un arc à flamme (22) pour fournir la chaleur, et avec un tube de sortie (5) au-dessus du niveau du bain de métal liquide, pour la vapeur provenant de l'intérieur du récipient (1), **caractérisé en ce que** le tube de sortie (5) débouche dans un compartiment (27) qui est maintenu à une température inférieure à la température de vaporisation, pour condenser le métal vaporisé, et **en ce que** plusieurs compartiments (27) avec une température descendante sont agencés en série, pour condenser différentes vapeurs de métal, le métal avec le point de vaporisation le plus haut est condensé dans le premier compartiment (27) et le métal avec le point de vaporisation le plus bas est condensé dans la dernière chambre.
